

Patented Feb. 26, 1946

2,395,688

# UNITED STATES PATENT OFFICE

2,395,688

## ALLOY STEEL

Luciano G. Selmi, Detroit, and Clarence L. Altenburger, Dearborn, Mich., assignors to National Steel Corporation, a corporation of Delaware

No Drawing. Application April 10, 1944,  
Serial No. 530,396

2 Claims. (Cl. 75—126)

This invention relates to improvements in low alloy steels. More particularly, the invention relates to steels of the type disclosed and claimed in our patents No. 2,234,130 issued March 1, 1941 and No. 2,250,505 issued July 29, 1941.

The subject matter of the present application includes certain subject matter appearing in our copending applications, Serial Nos. 460,272 and 460,273, both filed on September 30, 1942, and the present application is therefore in the nature of a consolidated continuation in part of the two copending cases.

In the steels described in the foregoing patents, zirconium is incorporated as a constituent to de-oxidize the steel and attain an inherently fine grain. In the present invention, by substituting vanadium for the zirconium in similar steels the many advantages of steels "A" of the patent have been retained while eliminating certain disadvantages inherent in the use of zirconium. These disadvantages in the use of zirconium in no way affect the characteristics of such steels but appear only during the manufacture. By the present invention similar steels incorporating the same characteristics as those of the steels "A" in the patents can be more easily produced, the substitution of vanadium for the zirconium eliminating many of the pouring and casting troubles encountered with the use of zirconium. On the other hand we have found that the incorporation of the vanadium in place of the zirconium does not deleteriously affect the physical characteristics of the specific steel involved. Thus the steel of the present invention has substantially the same physical characteristics as steels "A" disclosed in patents, No. 2,234,130 and No. 2,250,505.

The general object of the present invention is to provide a steel which may be easily and economically manufactured and which shall have important characteristics heretofore obtained only in steels using larger quantities of alloying metals.

More specifically referring to those alloys of the present invention wherein the carbon is maintained on the low side, the objects of the invention include provision for steels the compositions of which shall be variable within definite ranges in accordance with the size and shape of the finished steel; the provision of an improved high tensile steel for use in the "as rolled" condition or capable of being heat treated to predetermined and narrow ranges of hardness distribution or other physical properties dependent thereon. Referring more specifically to steels of the present invention where the carbon is maintained on the high side, other objects of the invention include the provision of steels resistant to high velocity impact, resistance to shock and fragmentation, and which shall have permanent high cohesion strength, the latter being in high ratio to

its shear strength to make the steel resistant to the growth and propagation of cracks. It is desirable that these steels have high degree or levels of hardness, variable hardenability, good ductility and machinability.

As is well known, many compositions of steel produced with laboratory facilities can be balanced chemically so as to produce physical properties within a given range. Such compositions may or may not be capable of yielding these same desired properties when subjected to the conditions prevailing in actual commercial steel manufacturing. Rolling temperatures, rate of cooling after rolling together with the size and shape of the finished material are the main variables affecting this condition.

In the specific case of those steels which have become known to the trade as low-alloy high tensile steels, in general they are required to possess tensile properties approximately as follows:

|                           |   |               |        |
|---------------------------|---|---------------|--------|
| Yield point               | — | p. s. i. min. | 50,000 |
| Tensile strength          | — | p. s. i. min. | 70,000 |
| Per cent elongation in 2" | — | per cent min. | 25     |

Many comparatively simple analyses are capable of producing tensile properties in the aforesaid range when rolled hot to comparatively thin gauges, by controlling finishing temperatures and by the use of copious application of water to the steel on the run out table or cooling bed after the steel has passed through the last stand of rolls. When the gauge or thickness of strip or plate, for example, increases, such procedures become rapidly less effective and tensile properties lower than the above minima are obtained from the steel in its rolled condition.

In the past few years the requirements of low alloy high tensile steels have increased swiftly. They were originally intended for relatively simple fabrication methods. Today such steels must weld by all commercial welding processes as easily as mild carbon steels; they must be equal to or better than mild carbon steels in the matter of deep drawing objects therefrom; they must be capable of responding to the ordinary methods of heat treatment and case hardening; they must possess good notched bar resistance at both normal and sub-normal temperatures, high fatigue resistance, especially fatigue resistance at notches or other stress-raisers which may reside within the body of the steel itself. The steel should have all contained nitrogen fixed in inactive forms and be free from strain or quench aging. The steel must not be air hardening at any carbon content and should possess no precipitable elements capable of impairing its physical properties upon stress relieving after welding or normalizing. This imposing list of properties demanded by modern steel users is due in part to the increasing precision of modern manufacturing and part-

ly to the increased use of technical testing of fabricated structures.

The steel of the present invention with the carbon on the low side has been found satisfactory within certain limits for fulfilling the above demands. A tabulation of the elements in this type of steel and their approximate percentages is set out below:

|                                        | Per cent    |
|----------------------------------------|-------------|
| Carbon                                 | .05 to .25  |
| Manganese                              | .50 to 1.00 |
| Silicon                                | .50 to .90  |
| Chromium                               | .25 to .75  |
| Vanadium                               | .01 to .20  |
| Phosphorus, maximum                    | .03         |
| Sulphur, maximum                       | .03         |
| Balance iron and incidental impurities |             |

When rolling temperatures are properly maintained on the lighter gauges and with accelerated cooling on the heavier gauges, the desired tensile properties can be achieved in the finished material. In stock of relatively small cross section, heat treatment by quenching and drawing is effective to produce a satisfactory hardenability and in such stock hardness distributions across heat treated sections can be controlled to predetermined and narrow ranges.

In the matter of carburizing it has been found that the case strength of the above steels after heat treating compare favorably with the highest types of alloy steels for carburizing known to the trade and the core hardness is satisfactory where too high a value is not required. In certain types of armor plate this is a matter of paramount importance. In such applications, one face of the steel plate to be fabricated into armor plate is carburized and the plate is then heat treated. It is required that the face not carburized be not too hard so that a bullet striking a carburized side will not effect cracking on the other side and throw off splinters or particles.

Steels of the present invention with the carbon maintained on the high side have characteristics and properties similar to high alloy steels which include appreciable amounts of nickel, for example. With the carbon on the high side the steels of the present invention have variable hardenability through unexpectedly wide ranges controllable by relatively small variations in the elements and by small changes of quenching temperatures. Such steels according to the present invention will have compositions within the following approximate ranges:

|                                        | Per cent |
|----------------------------------------|----------|
| Carbon                                 | .15-.70  |
| Manganese                              | .50-1.00 |
| Silicon                                | .50-.90  |
| Chromium                               | .25-.75  |
| Vanadium                               | .01-.20  |
| Phosphorus, maximum                    | .03      |
| Sulphur, maximum                       | .03      |
| Balance iron and incidental impurities |          |

A specific example of such steels with a carbon content of .48%, manganese .70%, silicon .75%, chromium .62%, vanadium .10%, phosphorus .09%, sulphur .021%, the remainder iron, will have a hardness in excess of 50 Rockwell C along a flat end quench bar up to  $\frac{1}{4}$ " from the quenching end when quenched from 1500° F. Such heat treatment includes holding an inch round bar at 1500° F. for an hour prior to quenching. The cooling rate is maintained at a rate in excess of 21° F. per second at 1250° F.

The higher carbon steels of the present invention may have the levels of hardness varied through large ranges by slight variations in temperature. The degree or levels of hardness may be varied materially by changes as small as 20° in quenching temperatures with shapes having comparatively thin or narrow cross sections. The steels may thus practically be treated to attain desired hardness levels throughout by variations of quenching temperatures through narrow ranges.

Throughout the range of carbon content in the present steels, nickel and copper may be present as residual elements. That is they may be present in the final steel because of forming an alloying element of the steel scrap employed in the production of the steel of the present invention. Where present as residuals, nickel may be in amounts up to approximately .10% and copper in amounts up to approximately .14%. Amounts of nickel up to .6% and copper up to .3% may occur in the steels of the present invention without materially affecting the property thereof, the nickel in the higher amounts perhaps adding some toughness, enhancing the heat treatment and adding somewhat to the corrosion resisting properties.

The steel of the present invention is inherently fine grained and substantially deoxidized.

We have found that in using the steel of the present invention for heat treated plates that certain optimum percentages of the constituents exist in accordance with the thickness of the plate. The following table shows some of these preferred compositions:

|                    | Plate thickness in inches |           |           |
|--------------------|---------------------------|-----------|-----------|
|                    | Up to $\frac{1}{4}$       | 1         | 2 and up  |
| Per cent carbon    | 0.15-0.50                 | 0.15-0.50 | 0.15-0.50 |
| Per cent manganese | .50-.75                   | .85-.95   | .90-1.00  |
| Per cent silicon   | .50-.90                   | .50-.90   | .50-.90   |
| Per cent chromium  | .50-.75                   | .60-.70   | .60-.70   |
| Per cent vanadium  | .01-.10                   | .01-.10   | .01-.10   |

From the foregoing description it will be seen that the applicants have produced a low alloy high tensile steel having its alloy elements selected, combined and balanced within narrow, but specific and critical ranges, whereby the improved steel having the characteristics and accomplishing the objects set forth is provided.

We claim:

1. A low alloy steel adapted for use as a high tensile steel and case carburizing purposes in the low carbon ranges and having improved heat treating properties in the higher carbon ranges, consisting of carbon up to about .70%, manganese about .70 to about 1.00%, silicon about .50 to about .90%, chromium about .50 to about .75%, vanadium about .01 to .10%, the balance being iron and incidental impurities.

2. A low alloy steel adapted for use as a high tensile steel and case carburizing purposes in the low carbon ranges and having improved heat treating properties in the higher carbon ranges, consisting of carbon up to about .50%, manganese about .85 to about 1.00%, silicon about .50 to about .90%, chromium about .60 to about .75%, vanadium about .01 to .10%, the balance being iron and incidental impurities.

LUCIANO G. SELMI.  
CLARENCE L. ALTBURGER.